

## UNITED STATES PATENT OFFICE

GEORGE G. THOMAS, OF ELIZABETH, AND LUDWIG J. CHRISTMANN, OF JERSEY CITY,  
NEW JERSEY, ASSIGNEES TO AMERICAN CYANAMID COMPANY, OF NEW YORK, N. Y.,  
A CORPORATION OF MAINE

## METHOD OF FLOTATION

No Drawing.

Application filed December 13, 1927. Serial No. 239,818.

This invention relates to the flotation of ores, more particularly to differential flotation involving the use of a cyanide. high we reduce the lime to a very small amount.

It has been well known for a number of years that sodium cyanide and other soluble cyanides when added to a mill circuit containing complex ores to be floated, acts as a depressant of some of the minerals, while allowing flotation of others. Cyanides are so used to a considerable extent in various types of ores, for example, ores containing copper and iron, where the cyanide inhibits the flotation of the iron allowing the copper to be removed as a concentrate.

By reason of the elimination of most or all of the lime in the first flotation operation, we then in the second stage, for the recovery of the iron, use only a very small amount of the acid such as sulphuric acid, thereby saving practically the entire cost of both lime and sulphuric acid. The amount of cyanide, for example, sodium cyanide, necessary for the operation is very small being from .10 to .20 pounds of sodium cyanide per ton of ore at a cost of approximately 2 to 4 cents per ton of ore compared to the cost of alkali and acid of about 22 cents per ton by the old process.

The general procedure has been to provide a mill circuit of ore, for instance, a low grade copper iron ore, in a suitable dilution with water and to add a substantial amount of lime to the circuit to make the same definitely alkaline. Suitable flotation reagents were added to the circuit and flotation of the copper, for example, was effected, either with or without the use of a cyanide. The remainder, containing most of the iron in the ore, was subjected to another flotation operation in the presence of an acid such as sulphuric acid.

In such a procedure, the lime was a considerable expense as, for example, an ordinary ore from Eastern Canada required about 10 pounds of lime per ton which, at say 1 cent per pound, meant a cost of reagent of 10 cents per ton.

In the second stage of the flotation it was necessary to add a large amount of sulphuric acid, say 30 pounds per ton, most of which was necessary to neutralize the lime originally added. This involved an expense of approximately 12 cents per ton. In a large operation, the cost of these reagents becomes very considerable.

We have found that contrary to the prior belief that a cyanide cannot be used in flotation circuits except in alkaline solutions, we operate in neutral or acid solutions with excellent results. By so doing we are enabled to entirely omit the addition of lime in most cases and in exceptional cases where the acidity of the mill solution is very

high we reduce the lime to a very small amount.

As an example of the operation of our invention, we took the above mentioned ore from Eastern Canada which required to float the copper 10 pounds of lime per ton in addition to the ordinary flotation reagents. We ran a series of tests on this ore, using no lime and adding small amounts of sodium cyanide in place thereof, together with Aero浮 #25 and pine oil as the flotation reagents. Aerofloat is the flotation reagent described and claimed in the patent to Whitworth #1,593,232, dated July 20, 1926.

The pH or hydrogen ion concentration of the mill solution was 6.8 to 7.0 which is a practically neutral solution. The results of the test showed that by the elimination of the lime and the addition of a small amount of sodium cyanide, the results obtained were at least as good as those obtained with the use of 10 pounds of lime per ton as shown by the following table:

| Test     | Reagents  |                    |               | Head      | Cu conc-    | Cu          | Recov-    | 90        |
|----------|-----------|--------------------|---------------|-----------|-------------|-------------|-----------|-----------|
|          |           |                    |               | assay     | cent        | tail        | ery       |           |
|          | Cu per    | Fe per             | Cu per        | Cu per    | Fe per      | Cu per      | Fe per    |           |
| Mill run |           |                    |               |           |             |             |           |           |
| 1.....   | NaCN 0.10 | Aerofloat #25 0.12 | Pine oil 0.02 | 2.4 29.0  | 20.0 31.0   | 0.30 29.0   | 0.00 0.0  | 95        |
| 2.....   | 0.15      | 0.08               | 0.022         | 2.92 29.6 | 15.86 22.58 | 37.10 29.60 | 0.23 0.33 | 27.3 29.6 |
| 3.....   | 0.20      | 0.08               | 0.022         | 7.93 29.7 | 24.47 22.47 | 32.70 32.70 | 0.39 0.39 | 6.11 29.4 |

Mill run reagents: lime 10.0#, T & T mixture 0.16#, pine oil, 0.022#, and xanthate 0.02#.

The iron flotation was conducted with the use of Aerofloat #25 and sulphuric acid in very small amounts giving the following results in a circuit having a pH of 5.2 to 5.4.

| Test | Reagents lbs./ton              |                | Fe concentrate |             | Tails       |             | Recovery    |             |
|------|--------------------------------|----------------|----------------|-------------|-------------|-------------|-------------|-------------|
|      | H <sub>2</sub> SO <sub>4</sub> | Aero-float #25 | Cu per cent    | Fe per cent | Cu per cent | Fe per cent | Cu per cent | Fe per cent |
| 10   |                                |                |                |             |             |             |             |             |
| 1.   | Mill run                       | 0.34           | 44.0           | 0.27        | 6.6         | Not given   |             |             |
| 2.   | 2.0                            | 0.35           | 45.2           | 0.09        | 5.9         | 5.4         | 70.4        |             |
| 3.   | 3.0                            | 0.08           | 0.50           | 47.5        | 0.08        | 3.1         | 9.4         | 85.1        |
|      | 3.0                            | 0.08           | 0.63           | 46.6        | 0.08        | 4.6         | 11.2        | 82.5        |

15 Mill run reagents: H<sub>2</sub>SO<sub>4</sub> 29.0#, coal tar-creosote 0.94#, xanthate 0.06# and pine oil 0.03#.

It will be seen that the recoveries were as good as had been previously obtained with very large amounts of sulphuric acid.

20 Another ore from one of the Southwestern States was tested in a similar manner, comparing the results obtained with the use of small amounts of sodium cyanide in a definitely acid solution with results obtained 25 by the use of lime in a definitely alkaline solution. The following table, denoting the copper flotation or recovery, shows that the cyanide flotation is superior to the lime flotation. The results show both better recoveries and lower tails.

| Test | Reagents lbs./ton |       | Concentrate assay |             | Tail assay Cu per cent | Cu recovery per cent | Fe elimination per cent | pH   |
|------|-------------------|-------|-------------------|-------------|------------------------|----------------------|-------------------------|------|
|      | NaCN              | CaO   | Aero-float #15    | Cu per cent |                        |                      |                         |      |
| 35   |                   |       |                   |             |                        |                      |                         |      |
| 1.   | None.             | None. | 0.115             | 18.45       | 15.8                   | 0.24                 | 78.1                    | 55.0 |
| 2.   | 0.10              | None. | 0.115             | 18.95       | 15.9                   | 0.13                 | 89.4                    | 53.5 |
| 3.   | 0.20              | None. | 0.115             | 18.30       | 16.0                   | 0.11                 | 90.4                    | 52.9 |
| 4.   | None.             | 2.0   | 0.115             | 20.95       | 18.3                   | 0.18                 | 83.9                    | 54.9 |
| 5.   | None.             | 4.0   | 0.115             | 21.25       | 19.4                   | 0.14                 | 87.5                    | 52.8 |
| 6.   | None.             | 6.0   | 0.115             | 21.80       | 18.9                   | 0.14                 | 87.5                    | 54.3 |

From the above examples of our invention it will be clear that we have discovered the important fact that a cyanide in very small amounts can be used to replace lime in the differential flotation of ores, where the circuits are neutral or acid, and that in circuits which had previously employed a cyanide in 50 alkaline solution, most or all of the lime may be omitted.

Previously, cyanide when used in flotation had been used only in alkaline circuits with the addition of lime in large amounts and 55 the results obtained were not markedly superior to those obtained by the present invention. This invention allows of a very large and considerable saving in cost of reagents which, in an industry which is highly competitive and in which profits are small, is an important factor.

We have tested our new method with other ores under varied conditions and have found 60 that equal and in some cases markedly superior results are obtained by our method to-

gether with the very material saving in cost of reagents. Our invention is, therefore, not limited to the specific examples set forth above, but includes various procedures involving the use of sodium or other soluble 70 cyanides in flotation circuits of neutral or acid character as set forth in the claims appended hereto.

What we claim is:

1. In the concentration of ores, the step 75 of subjecting the ores to froth flotation in an acid medium and in the presence of a single base cyanide.

2. In the concentration of ores, the step of 80 subjecting the ores to froth flotation in an acid medium and in the presence of a single base cyanide in amount not exceeding  $\frac{1}{2}$  lb. of cyanide per ton of ore.

In testimony whereof, we have hereunto 85 subscribed our names this 6th day of December, 1927.

GEORGE G. THOMAS.  
LUDWIG J. CHRISTMANN.

90

95

100

105

110

115

120

125

130